

# UNITED STATES PATENT OFFICE.

ISIDOR MARGOLIUS, OF NORFOLK, VIRGINIA.

## STUFFING OR PACKING.

1,182,697.

Specification of Letters Patent.

Patented May 9, 1916.

No Drawing.

Application filed January 22, 1916. Serial No. 73,752.

*To all whom it may concern:*

Be it known that I, ISIDOR MARGOLIUS, a citizen of the United States, and a resident of Norfolk, in the county of Norfolk and 5 State of Virginia, have invented a certain new and useful Improvement in Stuffings or Packings, of which the following is a specification.

My invention relates to improvements in 10 stuffings or packings, and it consists in the article of manufacture hereinafter described and more particularly pointed out in the appended claims.

An object of my invention is to produce a 15 cheap and efficient stuffing or packing to be used for stuffing mattresses, as packing material, as a heat insulating lining, etc.

A further object of my invention is to provide a stuffing or packing which is free 20 from objectionable odor.

A further object of my invention is to provide a stuffing or packing which is comparatively free from objectionable gum or other mucilaginous matter.

25 A further object of my invention is to provide a stuffing or packing which is substantially undecomposable in the presence of water.

Other objects and advantages will appear 30 in the following specification, and the novel features of the invention will be particularly pointed out in the appended claims.

In making experiments with the bark of the cypress tree, I have made certain discoveries in regard to the composition of the 35 same which one would not naturally expect. It is known that tanks made of cypress wood impart an odor and a taste to the water which is stored therein, and may even 40 impart a color. The bark of the cypress tree does not present from the outside an appearance to indicate its exceedingly fibrous nature, but I have found by experimenting that, this bark is composed of 45 fibers which are very loosely held together, so that by slight attrition or rubbing of the bark, the fibers may be separated.

In carrying out my invention, I may make use of any of a number of processes which 50 will produce a packing or stuffing having

the properties desired. It will suffice to mention one or two processes by means of which the object may be attained.

The bark is selected, and is first boiled to loosen the small amount of cementitious 55 matter which holds the fibers together. One may employ an alkali during this boiling, such as soda ash or soda lye, but such alkali is not absolutely necessary. The boiled bark is then dried, and may be passed 60 through rollers or through decorticating machines so as to break up the bark and to loosen up and separate the fibers. Instead of boiling the bark it may be treated dry. I have found that the fibers can be separated 65 merely by rolling them or twisting them, and therein the cypress bark differs from other fiber bearing plants which require to be combed in order to separate the fibers.

70 The fibers when separated are collected and form the stuffing or packing. This stuffing or packing, contrary to what might be expected, has no odor, and therein it differs from fibers, for instance, of pine 75 needles or other plants or woods which contain oils or rosin. One of the main properties of the packing composed of the fibers of the bark of the cypress tree is that it is practically undecomposable in the presence 80 of water, and for this reason, a mattress, for instance, which has become saturated with water, may be dried out and the packing will be in practically the same condition as before it was wet.

85 Packing made from the fiber of the bark of the cypress tree has a high luster, and in this respect it resembles hair. The packing is a good insulator of heat, and may be used as linings for refrigerators, and in fact, in 90 any case where a heat-insulating packing is necessary.

I claim:—

1. As an article of manufacture, a packing or stuffing material made solely from 95 the bast fibers of the bark of the cypress tree.

2. As an article of manufacture, a packing or stuffing which is substantially non-decomposable in the presence of water and 100

which is made solely from the bast fibers of the bark of the cypress tree.

3. A packing or stuffing which is non-decomposable and odorless, and which is 5 made solely from the bast fibers of the bark of the cypress tree.

4. A packing or stuffing, said stuffing be-

ing a heat insulator, non-odorous, and non-decomposable in the presence of water, said packing or stuffing being made solely from 10 the bast fibers of the bark of the cypress tree.

ISIDOR MARGOLIUS.

Copies of this patent may be obtained for five cents each, by addressing the "Commissioner of Patents.  
Washington, D. C."